

## UNITED STATES PATENT OFFICE

ROBERT R. FULTON, OF PITTSBURGH, PENNSYLVANIA, ASSIGNOR TO THE KOPPERS COMPANY, A CORPORATION OF DELAWARE

## PROCESS OF TREATING FABRIC

No Drawing.

Application filed June 7, 1927. Serial No. 197,236.

This invention relates to the treatment of fabric and more particularly to a process of coating or filling woven fabric with cellulosic material.

5 An object of my invention is to provide a coated or filled fabric of improved surface quality and strength.

10 A further object of my invention is to provide a process of coating or filling fabric with cellulosic material that is free from certain difficulties and disadvantages of the prior art.

15 My invention has for further objects such other operative advantages and results as may hereinafter be found to obtain.

20 The manufacture of coated and filled fabric is well known. The processes of the prior art have, in general, attempted to produce such material by spreading a solution 25 of cellulosic material, such as viscose, upon the fabric. The difficulties met with in these processes are not easily overcome. Viscose and other cellulosic solutions, such as a solution of cellulose in calcium thiocyanate solution, are viscous and the viscosity of such 30 solutions is subject to variation upon exposure to the atmosphere, temperature fluctuations, handling and the like. Consequently, it is very difficult to obtain layers of cellulosic material of uniform thickness. Constant care is required in spreading the cellulosic solution upon the fabric, and adjustments of feeding devices must be made very frequently.

35 The high viscosity of solutions of cellulose in calcium thiocyanate solutions makes it difficult to obtain thin layers therefrom. Thick layers are prone to crack and peel from the fabric base.

40 I overcome the difficulties and disadvantages of the prior art by spreading cellulosic pulp upon a fabric base and subsequently 45 accomplishing the partial solution or gelatinization of the pulp without, however, materially affecting the fabric base. I accomplish this object by coating the fabric base with cellulosic pulp, immersing the whole in a gelatinizing bath, such as a solution of calcium thiocyanate of regulated 50 strength, allowing the material to stand until

partial solution or gelatinization occurs, removing any excess of gelatinizing liquid and pressing and finishing the material in the usual manner.

55 In order that my invention may be clearly set forth and understood, I now describe, but without limiting my invention to such specific illustrative example, the preferred manner in which it is accomplished and performed.

60 A fabric base, which may consist of loosely woven cloth, is covered with a layer of pulp, such as sulphite pulp or cotton rag pulp, or other cellulosic material in finely divided state. The layer of cellulosic material may be of any desired thickness and may be applied to both sides of the fabric base or to only one side thereof, as desired. Spreading the cellulosic material upon the fabric base is easily accomplished in a manner 65 well known to those familiar with the art.

70 The fabric and the superimposed cellulosic pulp are more or less completely dried by passing them between hot squeezing rolls 75 whereby heat and pressure is applied thereto.

75 After leaving the rolls, the coated fabric is passed through a solution capable of effecting partial solution or gelatinization of the pulp. I prefer to use a solution of calcium thiocyanate having a boiling point of from about 134° to 140° C. and containing from 20% to 30% of 40% formaldehyde, but other calcium thiocyanate solutions and still 80 other gelatinizing solutions, or solvents, known to the art may be employed. With respect to the preferred solutions, I have found that beneficial results may be obtained by maintaining a temperature of 85 from 20° to 40° C. therein, but other temperatures may be employed, especially when solutions of different strengths or kinds are employed.

90 The fabric is preferably not permitted to remain in the gelatinizing bath for an extended period but is removed and squeezed by being passed through rolls or otherwise treated to remove any excess liquid which may have adhered thereto. The material 95 100

which now retains a sufficient amount of gelatinizing liquid to accomplish the desired result is allowed to stand for a predetermined period to permit gelatinization of the 5 pulp fibers. It may be wound upon a reel or folded or handled in any other convenient manner during this gelatinization period.

When the desired degree of gelatinization 10 is attained, the material is sprayed with water or subjected to the action of steam or otherwise treated to remove or dilute the gelatinizing agent and thereby coagulate the gelatinized material and the cloth is then 15 passed through warm squeezing rolls or other suitable apparatus whereby the gelatinized pulp is pressed into, and incorporated with, the fabric base. The cloth is then washed and dried in the usual manner.

20 According to the results desired, the raw materials of my process and the procedure thereof may be varied over a wide range, as will be apparent to those skilled in the art. For example, fabric bases woven from 25 flax, hemp, jute, or other fiber may be treated and the cellulosic pulp employed as filling or coating agent may be obtained from many sources.

Moreover, the sequence of steps may be 30 varied in carrying out the process of my invention. For example, under certain circumstances, it may be advisable to squeeze or press the coated fabric before spraying or steaming it to dilute the gelatinizing agent.

35 The nature of the product obtained in the process of my invention will vary according to the materials employed and also according to various other factors, such as the duration of the period of gelatinization.

40 Ordinarily, however, I prefer to allow gelatinization of the pulp to proceed to the greatest practicable extent without, however, materially affecting the fabric base. Partial gelatinization of the fabric base, however, is not necessarily a disadvantage as it 45 may assist in forming a bond between the base and the coating material.

The advantages of my process are at once 50 apparent to those skilled in the art. The difficulties of handling extremely viscous cellulosic materials that may be subject to fluctuations in viscosity are entirely obviated. The coating or filling which results is much more uniform and adherent and 55 will not crack or peel. Moreover, a considerable saving in chemicals is effected.

My process is not limited to the specific 60 examples given hereinabove by way of illustration but may variously be embodied within the scope of the claims hereinafter made.

I claim as my invention:

65 1. The process of treating fabric which comprises spreading cellulosic pulp over the fabric and then effecting a gelatinization of the pulp.

2. The process of treating fabric which comprises spreading cellulosic pulp over the fabric and subjecting the fabric and pulp to a liquid effective to gelatinize the pulp.

3. The process of treating fabric which 70 comprises spreading cellulosic pulp over the fabric, subjecting the fabric and pulp to the action of a cellulose solvent, allowing gelatinization of the pulp to take place and removing excess solvent.

4. The process of treating fabric which 75 comprises spreading cellulosic pulp over the fabric, immersing the fabric and pulp in a solution of calcium thiocyanate, removing the fabric and pulp and allowing them to 80 stand until the pulp is at least partially gelatinized but without materially affecting the fabric and pressing the gelatinized pulp into the fabric.

5. The process of treating fabric which 85 comprises spreading cellulosic pulp over the fabric, pressing and drying the fabric and pulp, immersing the dry material in a solution of calcium thiocyanate and formaldehyde, removing the treated fabric and pressing it to remove excess solution, allowing it to stand until gelatinization of the pulp occurs, removing the remaining solution and washing and drying the coated fabric.

6. The process of treating fabric which 95 comprises spreading finely divided cellulose over the fabric, subjecting the whole to the action of a cellulose solvent until gelatinization of the applied cellulose is effected and then coagulating the gelatinized cellulose.

In testimony whereof, I have hereunto 100 subscribed my name this 2nd day of June, 1927.

ROBERT R. FULTON.

105

110

115

120

125

130